

# UNITED STATES PATENT OFFICE.

JESSE B. HODGES, OF SALEM, ARKANSAS, ASSIGNOR OF ONE-HALF TO  
JOHNSON P. WOODS, OF SAME PLACE.

## COMPOSITION FOR TANNING.

SPECIFICATION forming part of Letters Patent No. 526,229, dated September 18, 1894.

Application filed February 24, 1894. Serial No. 501,429. (No specimens.)

*To all whom it may concern:*

Be it known that I, JESSE B. HODGES, of Salem, in the county of Fulton and State of Arkansas, have invented a new and useful 5 Composition for Tanning Hides, of which the following is a full, clear, and exact description.

This invention consists in a new composition of matter for tanning hides, substantially 10 as hereinafter described and pointed out in the claims.

Prior to tanning, I soak the hides till soft and remove all flesh. Hard hides ought to be worked over on the flesh side to soften them. 15 The hides are then limed in the following way: I take twenty (20) gallons of water and add about twenty-two (22) quarts of slaked lime, and handle the hides in said solution several times the first two days and afterward once a day till the hair is made removable. I then remove the hair and flesh. The 20 hides are then ready for the bate which is prepared as follows: To twenty (20) gallons of water add one bushel of wheat bran and one peck of hen manure, the whole to be 25 plunged well, when the bate will be ready for use. In the bating operation, the hides should be handled several times a day till free of lime; they will thus become soft and limber; 30 they are then thrown on a table and worked over on the flesh side with a steel knife or rubber, and on the grain side with a stone knife or rubber; they are then scoured with clean water, when they will be ready for the 35 tan. The tanning liquor, to which the hides are then subjected, consists of about twenty gallons of water having dissolved in or mixed with it five pounds of the extract of palmetto root, half a pound of stramonium, two pounds 40 of gambia and five pounds of salt. In this

liquor, the hides are to be plunged well, and handled once a day till the grain is tanned. Five pounds of the extract of palmetto root should be added each day till the hides are well tanned. The hides are then taken out 45 of the tanning vat and scoured well, till the ooze or remaining liquor in them is removed, then hung in the shade till half dry, then the grain sides of the hides are oiled, and afterward the flesh side of them is stuffed with oil 50 and tallow in equal parts, mixed. This puts the tanned leather in condition ready for finishing.

The palmetto or saw palmetto, the extract of the roots of which is used in the above described tanning liquor, is of abundant growth in many parts of the coast portions of the United States, and one cord of these roots contains about as much tanning property as two cords of the best oak bark, and the same can 55 be gathered at a very inconsiderable expense. Said roots can be crushed and their essence extracted for much less than the best oak bark extract can be obtained.

By the process herein described, light hides 60 will tan in two days and the heaviest of hides in twenty days, and at a cost of about three cents per pound to the tanned leather.

Having thus fully described my invention, I claim as new and desire to secure by Letters 70 Patent—

The herein described composition for tanning leather, consisting of water, extract of palmetto root, stramonium, gambier and salt, in about the proportions specified.

JESSE B. HODGES.

Witnesses:

JOHN C. FEULNER,  
W. M. CASTLEBERRY.